

Aug. 6, 1935.

G. I. PUTNAM ET AL

2,010,320

PROCESS FOR DYEING RAYON KNIT PIECE GOODS

Filed Jan. 12, 1929



Inventors

George Ires Putnam and Clifford Fisher Worthen  
By their Attorneys

Warfield & Watson

## UNITED STATES PATENT OFFICE

2,010,320

PROCESS FOR DYEING RAYON KNIT  
PIECE GOODS

George Ives Putnam and Clifford Tasker Worthen,  
Utica, N. Y., assignors to McLoughlin Textile  
Corporation, Utica, N. Y., a corporation of New  
York

Application January 12, 1929, Serial No. 332,074

18 Claims. (Cl. 8—5)

The invention relates to a process of dyeing and more particularly to the dyeing of rayon with vat dyes and includes correlated discoveries and improvements whereby and wherewith the dyeing of rayon is enhanced.

An object of the invention is to provide a process by which rayon may be dyed fast shades with the various classes of vat dyes so that the colors will not be affected by the usual agencies as light, 10 washing, etc.

Another object of the invention is to provide a process for dyeing rayon in the form of knit piece goods a variety of shades with vat dyes.

A further object of the invention is to provide a 15 process whereby rayon knit piece goods may be dyed fast shades commercially in an economical manner in large quantities in a dyeing machine.

Furthermore it is an object of the invention to provide a process for dyeing rayon knit piece goods with vat dyes giving fast to light and washing shades with not only a retainment of the inherent qualities of the rayon, but with an enhancement of their desirable properties.

Other objects of the invention will in part be 20 obvious and will in part appear hereinafter.

The invention accordingly comprises the several steps and the relation and order of one or more such steps with respect to each of the others, and the apparatus embodying features of construction combinations of elements and arrangement of parts which are adapted to effect such steps, all as exemplified in the following detailed disclosure, and the scope of the application of which will be indicated in the claims.

For a fuller understanding of the nature and objects of the invention reference should be had to the following detailed description taken in connection with the accompanying drawing, in which the figure represents a side elevation, partly 25 broken away, of a dyeing machine suitable for carrying out the dyeing operation. This machine consists of the usual tub 1, which is provided with a perforated partition 2 for maintaining the knit piece goods 3 out of direct contact 30 with the wall of the tub and so curved as to render the reeling or working of the goods easy. The sides and ends of the tub are provided with suitable outlets 4 for the overflow of the liquid during the washing operation. Positioned above the 35 tub are driving gears 6 and 7, a carrying roll 8, a large reel 9 and a small reel 10. The roll 8 is an idling roll. The reels 9 and 10 are driven by a chain 11 and a belt 12, respectively. The reel 10 is much smaller than the reel 9.

In the dyeing operation the goods is worked

over the large reel previous to the introduction of the vat dye, and is removed from the large reel and passed over the small reel 10 just before introducing the dyestuff or coloring material. The drive of the small reel is such that it travels at a rate which is about 10% faster than that of the large reel, and being of small diameter, the goods is reeled through the liquor in the tub more rapidly whereby the time of exposure to the air is materially lessened. The tub is also provided with a pipe not shown in the drawing by means of which wash water is introduced when the dyeing operation has been completed.

In the practice of the invention the dyeing machine is filled to the proper level with water 15 to which an alkali and a retarding agent are added. Into this bath the rayon knit piece goods is introduced and worked therethrough in the cold until the goods is thoroughly saturated with the bath liquor. This is desirable in order to 20 obtain level shades. When the goods is saturated, which may require a period of about twenty minutes, a reducing agent is added, and when well distributed throughout the bath, the vat dyestuff for the shade desired is added in the 25 reduced condition, i. e., the dyestuff has been suitably reduced before introduction into the bath containing a reducing agent in order that the reduced condition may be maintained.

The working or reeling of the goods through 30 the bath is continued with increase of temperature until the dyestuff is fixed by the fiber. The increase in temperature is gradual and reaches at least 100 degrees F., whereupon it is maintained throughout the dyeing operation. The 35 dyeing having been completed, wash water is introduced with reeling of the goods being continued until the dyeing solution is removed from the fiber. It is not desirable to dump the dye bath and then to wash, but rather it has 40 been found more satisfactory to introduce the wash water into the bath in the form of a spray and allow the liquid to run off through the overflows provided therefor about the tub. When the washing is completed, the dyestuff is oxidized 45 by running in a bath containing an oxidizing agent such as hydrogen peroxide, sodium perborate or other suitable oxidizing agent, and is finished by a soaping in hot solution. The goods is then dried, whereupon it is ready for manufacture into various garments or other articles.

There are various methods by which rayon is manufactured. Those mostly used are the viscose, the copper ammonia, the nitrocellulose and the cellulose acetate. The first three methods 50

- yield a rayon which is, as it were, a regenerated cellulose, whereas the last yields a rayon which is a cellulose ester. These two types of rayon, while differing in their chemical composition, 5 may nevertheless be dyed according to this invention in the same way. It is to be observed, however, that the effect of an alkali will be somewhat different upon the two types of fiber. In the case of the viscose, copper ammonia and 10 nitrocellulose rayon, an alkali, as caustic soda, will have, in addition to the effect during the dyeing operation, a beneficial action upon the structure of the rayon, which gives to the finished material, a special soft, velvety, silk-like 15 feel and finish. When dyeing a cellulose acetate rayon, in order to retain the characteristic properties of this type of rayon, attention should be given to the fact that inasmuch as cellulose acetate is an ester, it is therefore capable of 20 saponification by an alkali, and care is to be exercised so that the amount of alkali used in the dye bath is not sufficient to materially affect or saponify the cellulose acetate. Should this care not be exercised, the rayon produced will have 25 the characteristics rather of the viscose type than of the cellulose acetate type.
- The vat dyes or coloring matters, which are used in a reduced condition, are those belonging to the indigoid, carbazol and anthraquinone 30 classes.
- The method of procedure in general is that a bath is prepared in the tub of the dyeing machine containing an alkali, such as caustic soda, or caustic potash, and a retarding agent which 35 may be a sulphite waste liquor product or derivative. The rayon knit piece goods are run in this bath for a period sufficient to thoroughly saturate the goods, in order to insure level dyeing. This preliminary treatment with the retarding agent is of importance in preventing the 40 dye-stuff when added from going into the cloth to rapidly with the result that the dye-stuff would tend to deposit itself unevenly upon the cloth due to its too rapid exhaustion. The preliminary treatment of the goods with the retarding agent thus acts to provide for particularly 45 level dyeing. A period of twenty minutes has been found to give satisfactory results. To this bath is then added the required amount of retarding agent as sodium hydrosulphite, and when 50 this agent has been well distributed throughout the bath, there is added the desired vat dyestuff previously reduced. The preparation of the dye solution may be made by dissolving the required 55 quantity for the shade to be produced in water containing sodium hydrosulphite and caustic soda or caustic potash. The contents are stirred until reduction is completed, whereupon it is ready for use in the dye bath. In dyeing the knit 60 piece goods, the dye bath should at all times be in a reduced state. Otherwise imperfect and non-level shades will result.
- The dyeing operation is started in the cold, and 65 the goods, which has previously been reeled by passing over the roller 8 and the reel 9, is now passed over the roll 8 and the reel 10 in order to reduce the time of exposure to air and thus to decrease the tendency to oxidation, and the temperature is gradually raised to that required for 70 the particular dyeing operation. The reeling of the piece goods is continued at this temperature, which may vary from 100 to 160 degrees F., depending upon the material and the dyestuff being used, until the desired shade is obtained. The goods are then washed free of the bath liquor

75 by a spray of water entering beyond the perforated partition at the left of the dyeing machine and flowing out through the overflows at the sides and ends of the tub. The washing is continued until the dye liquor is thoroughly removed, whereupon the goods is oxidized by passage through a bath which may contain hydrogen peroxide as the oxidizing agent. The operation is completed by a soaping in hot solution, for example at a temperature of 180 degrees F. in order 10 to fully develop the shade and to impart fastness. The goods may then be dried and utilized in the manner desired.

More in particular, but also a general formula, the dyeing of 400 pounds of rayon knit piece 15 goods may be accomplished in a bath containing the vat dye in the percentage for the shade to which the work is directed: 900 to 1000 gallons of water; 9 to 20 pounds of caustic soda; 7 to 12 pounds of sodium hydrosulphite; and 1 to 4 20 pounds retarding agent, as a sulphite waste liquor product. It has been found that within the limits here given, practically any shade may be obtained on rayon knit piece goods with vat dyes. It may be mentioned, however, that the quantities of 25 caustic soda, sodium hydrosulphite and retarding agent will vary somewhat with the various dyes and the best results must be ascertained for each. Also the ability of the rayon to fix or take up the various vat colors varies, and 30 the dyeing conditions are to be adjusted in order to obtain the best results with respect to this factor.

The examples hereinafter given present illustrative details of procedures adapted for use with 35 particular dyes pursuant to the foregoing:

#### Example I

Rayon knit piece goods may be dyed a coral shade with the indigoid vat dye ciba scarlet G 40 (color index No. 1228) extra powder in an amount of 1% by utilizing 1000 gallons of water in which is dissolved 10 pounds of caustic soda, 10 pounds of sodium hydrosulphite, and 3 pounds of the sulphite waste liquor product. 400 pounds of rayon 45 knit piece goods may be dyed by the procedure indicated, starting cold, and gradually increasing the temperature to 110 degrees F.

#### Example II

Rayon knit piece goods may be dyed a honeydew shade by using an orange carbazol vat dye in paste form in an amount of  $\frac{3}{4}\%$  with the use of 10 pounds of caustic soda, 8 pounds of sodium hydrosulphite, 3 pounds of the sulphite waste liquor product, and 1000 gallons of water. Four hundred pounds of rayon knit piece goods are dyed in this bath, being entered cold and the temperature gradually raised to and maintained at 160 degrees F.

#### Example III

Rayon knit piece goods may be dyed a nile green shade by the use of a mixture of anthraquinone vat dyes, for example, an anthraquinone green vat dye in paste form in an amount of  $\frac{3}{8}\%$  and an anthraquinone yellow vat dye in powder form  $\frac{1}{4}\%$  utilizing 1000 gallons of water, 70 20 pounds of caustic soda, 10 pounds of sodium hydrosulphite, and 3 pounds of the sulphite waste liquor product. 400 pounds of rayon piece goods are dyed. The temperature is gradually raised to and maintained at 120 degrees F.

## Example IV

Cellulose acetate rayon knit piece goods may be dyed a scarlet shade with a red indigoid vat dye in an amount of  $\frac{1}{2}\%$  utilizing 700 gallons of water, 7 pounds of caustic soda, 6 pounds of sodium hydrosulphite and 2 pounds of the sulphite waste liquor product. 200 pounds of cellulose acetate rayon are reeled, being entered cold, and the temperature gradually raised and maintained at 140 degrees F. When the dyeing is completed the washing, oxidizing and soaping is as previously described.

Vat dyes of the carbazol and anthraquinone classes may be used for the dyeing of cellulose acetate rayon. For example, if a violet shade is desired, it may be obtained by dyeing in a bath containing a violet carbazol vat dye powder, and if a blue shade, it may be developed in a bath containing a blue anthraquinone vat dye.

As exemplifying other vat dyes which may be used, more particularly with rayon of the viscose, copper ammonia and nitrocellulose types, mention may be made of carbazol and anthraquinone dyes.

It is to be understood that sulphite waste liquor derivatives are included under the terms "sulphite waste liquor product" and "sulphite waste liquor" etc. as used herein.

Since certain changes in carrying out the above process and in the constructions set forth, which embody the invention may be made without departing from its scope, it is intended that all matter contained in the above description or shown in the accompanying drawing shall be interpreted as illustrative and not in a limiting sense.

Having described our invention, what we claim as new and desire to secure by Letters Patent, is:

1. A process of dyeing, which comprises working rayon knit piece goods in a bath containing an alkali and a retarding agent, subsequently adding a reducing agent and a vat dye in reduced condition, continuing the working until the dye has been fixed, and then washing and oxidizing.

2. A process of dyeing, which comprises working rayon knit piece goods in a bath containing an alkali and a retarding agent for about twenty minutes, subsequently adding a reducing agent and a vat dye in reduced condition, continuing the working until the dye has been fixed and then washing and oxidizing.

3. A process of dyeing, which comprises working rayon knit piece goods in a bath, in the cold, containing an alkali and a retarding agent, subsequently adding a reducing agent and a vat dye in reduced condition, continuing the working with increase of temperature until the dye has been fixed, and then washing and oxidizing.

4. A process of dyeing, which comprises working rayon knit piece goods in a bath, in the cold, containing an alkali and a retarding agent for about twenty minutes, subsequently adding a reducing agent and a vat dye in reduced condition, continuing the working with increase of temperature until the dye has been fixed, and then washing and oxidizing.

5. A process of dyeing, which comprises working rayon knit piece goods in a bath, in the cold, containing an alkali and a retarding agent for about twenty minutes, subsequently adding a reducing agent and a vat dye in reduced condition, continuing the working with increase of temperature until the dye has been fixed, then washing and oxidizing, and soaping in a hot solution.

6. A process of dyeing, which comprises reeling rayon knit piece goods through a bath, in the cold, containing a caustic alkali and a sulphite waste liquor product as a retarding agent for about twenty minutes, subsequently adding sodium hydrosulphite and a vat dye in reduced condition, continuing the reeling with increase of temperature until the dye has been fixed, and finally washing, oxidizing and soaping in hot solution. 10

7. A process of dyeing, which comprises working rayon fabric for a period of time in a bath containing an alkali compound and a retarding agent, and thereafter including in said bath a vat dye and a reducing agent, and continuing the 15 working.

8. A process of dyeing, which comprises working rayon fabric for a period of time in a bath containing an alkali compound and a retarding agent, and thereafter including in said bath a vat 20 dye in reduced condition and a reducing agent, and continuing the working.

9. A process of dyeing, which comprises working rayon fabric for a period of time in a bath containing an alkali compound and a retarding 25 agent, and thereafter including in said bath a vat dye and a reducing agent, and continuing the working, the retarding agent being in the proportion of .01 to .04 pound to each 9 to 10 gallons of water. 30

10. A process of dyeing, which comprises working rayon fabric for a period of time sufficient to thoroughly saturate the goods in a bath containing an alkali and a retarding agent, and thereafter including in said bath a vat dye and a 35 reducing agent, and continuing the working.

11. A process of dyeing, which comprises working rayon fabric for a period of time sufficient to thoroughly saturate the goods in a bath containing an alkali and a retarding agent, and thereafter including in said bath a vat dye and a reducing agent, and continuing the working with increase in temperature. 40

12. A process of dyeing, which comprises working rayon goods in a bath containing an alkali 45 and a retarding agent, subsequently distributing a reducing agent throughout said bath and thereafter adding a vat dye in reduced condition and continuing the working until the dye has been fixed, and then washing and oxidizing. 50

13. A process of dyeing, which comprises working rayon goods in a bath containing an alkali and sulphite waste liquor, subsequently distributing a reducing agent throughout said bath and thereafter adding a vat dye in reduced condition and continuing and working until the dye has been fixed, and then washing and oxidizing. 55

14. A process of dyeing, which comprises working piece goods in a bath containing an alkali and a retarding agent, and subsequently including 60 in the bath a reducing agent and a vat dye in reduced condition.

15. A process of dyeing, which comprises working piece goods in a bath containing an alkali and a sulphite waste liquor product, and subsequently 65 adding a reducing agent and a vat dye in reduced condition.

16. A process of dyeing, which comprises working piece goods in a bath containing an alkali and a sulphite waste liquor product, subsequently 70 adding a reducing agent and a vat dye in reduced condition, continuing the working with an increase in temperature until the dye has been fixed, and then washing and oxidizing.

17. A process of dyeing, which comprises work- 75

ing piece goods in a bath containing an alkali and a sulphite waste liquor product for about twenty minutes, subsequently adding a vat dye in reduced condition, continuing the working in 5 the presence of a reducing agent with an increase of temperature until the dye has been fixed, and then washing and oxidizing.

18. A process of dyeing, which comprises working piece goods in a bath containing an alkali 10 and a retarding agent, and subsequently including

in the bath a reducing agent and a vat dye in reduced condition, and which involves utilizing the ingredients in the following proportions with respect to each nine or ten gallons of water: sulphite waste liquor product .01 to .04 pound, caustic soda about .09 to .2 pound, sodium hydrosulphite about .07 to .12 pound, and a vat dye in suitable proportion.

GEORGE IVES PUTNAM.  
CLIFFORD TASKER WORTHEN. 10